

# UNITED STATES PATENT OFFICE.

JOHN J. C. SMITH AND MICHAEL SMITH, OF PASSAIC, NEW JERSEY.

## VULCANIZATION OF RUBBER COVERINGS FOR ELECTRICAL CONDUCTORS.

SPECIFICATION forming part of Letters Patent No. 317,587, dated May 12, 1885.

Application filed August 1, 1884. (Specimens.)

*To all whom it may concern:*

Be it known that we, JOHN JOSEPH CHARLES SMITH and MICHAEL SMITH, citizens of the United States, residing at Passaic, in the county of Passaic and State of New Jersey, have invented certain new and useful Improvements in Vulcanizing Rubber or other Vulcanizable Insulation Compounds used as Coverings of Electric Conductors, of which the following

10 is a specification.

The object of this invention is to vulcanize such coverings in such a manner as to avoid the detrimental effects of moisture on the insulating-coverings of electric conductors while such coverings are in process of vulcanization.

15 We have found that any moisture which may come in direct contact with the insulating-covering of electric conductors while such covering is being vulcanized will seriously affect 20 and impair, if it does not destroy, the insulating qualities of the covering.

In order that those who are skilled in the art of producing highly-insulated electric conductors may fully understand the novelty and 25 importance of our invention, we will first relate some facts which came within the scope of our observation while going through a long series of experiments on an extensive scale for the purpose of producing a high insulation of 30 electric conductors by the use of a vulcanized-rubber compound.

Under the principal methods now used to vulcanize the covering of electric conductors, either the insulating compound is made so that 35 it may be vulcanized in a dry-heat chamber, where no pressure can be applied to the compound during the process of vulcanization, or the covered conductors are packed in dry soap-stone-powder and are placed in a vulcanizing-40 vessel, where steam is admitted, which produces the required heat and pressure at the same time. The last-named is very troublesome on account of the difficulty of properly packing a long piece of insulated wire in the 45 soapstone. In both cases the compounds used as insulating-coverings are made up with a view to being of such nature that they can be vulcanized in either one or the other way, and therefore are not of such high insulating qualities as they otherwise might be. Many slight

modifications of these systems are in use; but the principles remain the same.

While carrying on our experiments we used both of these systems and many of the sundry modifications in vogue; but found invariably 55 that the insulation resistance of the compounds was very much lower after vulcanization than before, and too often was lost altogether. By close observation we found that the compound absorbed more or less moisture during vulcanization by one or the other mode. When vulcanized in dry heat without pressure, the compound was full of fine pores unless it was mixed in considerable quantity with heavy ingredients not suitable for producing high insulation. Such observation led us to adopt 65 our present new method, the principle of which is to inclose the insulating-covering in a hermetical envelope, through which moisture cannot penetrate under pressure, and to vulcanize 70 the covering under such a protection. This effectually prevents moisture from coming in contact with the compound while it is being vulcanized.

We have carried our invention into effect 75 with complete success in the following manner: We lay a sheet of the insulating compound firmly on a long sheet of heavy tin-foil, and then cut both in long narrow strips, in the manner described by J. J. C. Smith in his 80 Patent No. 276,725, dated May 1, 1883, with reference to cutting in long strips combined sheets of insulating and fibrous material. Such strips of tin-foil, in combination with the vulcanizable insulating material, we lay on the 85 wire by means of the covering-machine described and claimed by the said J. J. C. Smith in his Patent No. 276,724, dated May 1, 1883.

Under our present invention the tin-foil answers the same purpose as the fibrous sheet 90 in affording facility for laying and pressing the covering closely on the wire; but in addition to this it serves the very important purpose of providing an impervious envelope for the insulating-covering, and protecting it fully 95 against the influence of moisture during vulcanization, thus permitting the direct pressure and heat of steam without injurious effect. It also differs from the fibrous covering in that it does not become inseparably incorporated 100

with the insulating-covering. It has long been known that all vulcanizable compounds become much better and of closer texture if vulcanized under pressure. Many cannot be vulcanized 5 in a solid condition without pressure. Others which can be vulcanized in dry heat without pressure possess this capability because heavily loaded with ingredients injurious to a good insulation.

10 When the insulating-cover is to be vulcanized, we coil the covered wire on a large but light metallic reel in two or three layers. This reel is so arranged that it may be put readily in and out of the vulcanizer, and that it can 15 be revolved horizontally in the vulcanizer while the same is closed and in operation. The revolving of the reel is accomplished by means of a shaft extending through a stuffing-box in the head of the horizontal vulcanizer 20 and provided with a driving-gear on the outside.

The reel may be advantageously made to contain about two miles of wire at one charge, and is rotated for the purpose of continually 25 changing the position and weight of the wire and its covering, which keeps the wire central in the covering while it is softened by heat before the vulcanization takes place.

When the vulcanization is completed, the 30 wire is taken out, and the tin envelope, having performed its function, is removed from the insulating-covering, leaving a smooth and dense surface.

To illustrate the importance of a tin-foil or 35 other metallic foil covering on the outside of the insulation-covering as a protective envelope during vulcanization, we will state the results of a number of experiments in vulcanization by other methods, and the results when 40 we used the metallic envelope.

An insulation compound such as is used in one of the best-known manufactories of insulated wire, and which we designate as "compound No. 1," was laid one twenty-fourth of 45 an inch thick on one thousand feet of No. 14 copper wire. Before vulcanization the insulation resistance of the cover was one hundred and eight megohms. It was then vulcanized in a dry-heat chamber without pressure. After 50 vulcanization the insulation resistance of the covering stood only twenty-seven and one-half megohms, and it fell to fifteen megohms after immersion in water for three days. This proved that fine pores must have formed during 55 vulcanization, which absorbed moisture, thereby injuring the insulation. Another one thousand feet of wire, covered with the same compound No. 1 one twenty-fourth of an inch thick, showed one hundred and twelve megohms before vulcanization. It was vulcanized in a dry soapstone-powder bed carefully packed and heated under steam-pressure. After vulcanization the insulation resistance of this covering was thirty-seven and one-half 60 megohms. Three days immersion in water brought it down to twenty-three megohms. A third piece one thousand feet long was cov-

ered with the same compound No. 1 to the same thickness, and was protected by what is commonly called a "water-proof tape." This 70 piece was vulcanized in steam under pressure in the manner in which soft-rubber goods are generally cured. After vulcanization it showed only seven megohms insulation, and in less than three hours immersion in water 75 it came down to one-half megohm. A fourth piece of one thousand feet was covered with the same compound the same thickness, but protected by our metallic envelope. Before 80 vulcanization this piece indicated one hundred and thirteen megohms insulation resistance. It was vulcanized in steam under sixty pounds pressure. After vulcanization this piece indicated an insulation resistance of one hundred and sixty-three megohms, which 85 showed a great increase of the insulation resistance. Three days immersion in water proved it to be unalterable.

The rubber compound described and claimed in J. J. C. Smith's application filed the 7th of 90 April, 1884, showed still more remarkable results. This compound is absolutely water-proof and one of the best insulators. It was laid on one thousand feet of No. 14 copper wire, one twenty-fourth of an inch thick, the 95 same thickness as in the previous experiments with compound No. 1. When raw, this compound showed an insulation resistance of two hundred and forty megohms. After vulcanization in dry soapstone-powder under pressure of steam, it showed an insulation resistance of ninety-two megohms, falling to forty-seven after three days immersion. A second piece covered with the said Smith's compound and with water-proof tape as a protection, and 100 vulcanized in steam under pressure, showed only seventy-two megohms insulation after 105 vulcanization, falling to forty megohms after three days immersion in water. A third piece of one thousand feet of wire covered with 110 Smith's compound, but protected by our metallic envelope, was vulcanized in steam under pressure. After vulcanization it showed an insulation resistance of five hundred and seventy megohms. Immersion in water for 115 weeks had no influence upon it. Repeated trials with the same compounds and many others showed corresponding results, proving the fact that if an electric conductor insulated with a vulcanizable compound is covered with 120 a metallic envelope in the manner described, and is vulcanized under such a protection, the insulation resistance of the covering is very much improved. All the named trials were made with equal accuracy, and all tests and 125 measurements taken with the most sensitive instruments and galvanometers.

In order to avoid any possibility of mistake about one or the other compound, we took hard-rubber or ebonite compound, which is known 130 as one of the best insulators. It was laid on the wire the same thickness as the other. The first sample vulcanized in dry soapstone showed an insulation resistance of ninety-seven

megohms, but fell to forty after immersion. The second example vulcanized in steam showed only one-half megohm after vulcanization. The third sample was vulcanized under the protection of the metallic envelope. After vulcanization it stood two hundred and eighty megohms, and did not change by immersion in water. These trials proved conclusively that all vulcanizable compounds suffer in their insulating qualities when vulcanized in such a manner that moisture may come in contact with the material in process of vulcanization. If vulcanized in dry heat or soapstone, it suffers from want of pressure on the compound, and a fine porous formation takes place, or the compound must be so much loaded with other ingredients as to affect its insulating qualities.

We are well aware that tin-foil or other metallic sheets are used in the manufacture and vulcanization of rubber goods to obtain smooth surfaces, or to keep the rubber in shape, or to facilitate molding and pressing in special forms; but it will be apparent that the impervious metallic envelope performs an essentially different and novel function in our process of

vulcanizing insulation-coverings of electrical conductors.

We use the tin-foil or other pliable metal sheets as an envelope that cannot be penetrated by moisture, so that we may fully protect our insulating compound against the detrimental influence of moisture while it is vulcanized, permitting us to use direct action of steam as the best and most convenient medium to produce the required heat and pressure at the same time.

What we claim as new, and desire to secure by Letters Patent, is—

The mode or process herein described of vulcanizing the insulating-covering of electrical conductors, the same consisting in enveloping the covered wire in a tight and impervious cover of tin-foil or other pliable metal, and subjecting it to the combined and simultaneous action of heat and pressure.

J. J. C. SMITH.  
MICHAEL SMITH.

Witnesses:

JOHN B. PUDNEY,  
EUGENE C. SMITH.